

## UNITED STATES PATENT OFFICE

TATSUO WAKABAYASHI, OF NEW YORK, N. Y.

## INKING MEANS

No Drawing.

Application filed July 24, 1929. Serial No. 380,759.

The present invention aims to provide a novel and improved composition of matter in the nature of a plastic mass for use as the working portion of an inking or stamp pad, 5 to mention one utilization of the invention now especially in mind.

Otherwise stated, the subject of the invention is a new and valuable combination of ingredients, constituting by their intermingling and interpenetration a mass of material which may be plastically applied and compressed within a cup-like holder or spread on a supporting surface, and then employed, for instance, exactly as in the familiar cloth 15 or felt covered and ink soaked pad proper of a so-called stamp pad.

An important object of the invention, then, in a more limited aspect of the latter, is to provide a novel and improved pad proper, 20 particularly useful in connection with a container of the familiar flat, tray-like, hinged-cover type, to fill or substantially fill such container or an appointed compartment therein; such containers, as is well known, being commonly used as carriers for stamp pads proper, and hence being generally called stamp pads.

A broad object of the invention is to employ an indiscriminately but substantially uniformly intermingled mass of fibrous material, and preferably such a mass including a plurality of fibres of dissimilar origin, whereby a quasi-felted, that is, an enduringly plastic and at the same time an enduringly 35 elastic mass may be provided once there has been incorporated therein, in addition to said fibrous material or materials to act as the base, various binding and inking substances or materials intermingled with each other 40 and with the base in such manner as to be uniformly dispersed or distributed between and within the fibres of the base; all to result in the provision of a new and valuable composition of matter which will keep indefinitely, which may be applied plastically 45 to a flat support or compressed within a shallow or other suitable container, which will then adhere to such support or container, which will have a continuing elasticity, 50 which thereafter and for a very long time

will not dry up, or require replenishment of the inking substance or material, or become permanently distorted under repeated forcible applications thereto of a stamp or other printing instrumentality to be inked thereby 55 preparatory to a printing operation of such instrumentality, and which, when desired, may without difficulty be removed from the base or tray supporting or confining the same and hence may readily be transferred to another base or tray or other suitable support or location.

These and various other objects and advantages of the invention will become apparent hereinafter or will be specifically referred to as this specification proceeds.

Referring now in detail to the new composition of material, its ingredients and mode of manufacture:

I have discovered that sponge fibre, and particularly vegetable sponge fibre produced preferably from vegetable sponges as below explained, especially when mixed with moxa so that an indiscriminate and substantially uniform intermingling of the dissimilar 70 sponge and moxa fibres results, provides a permanently inherently elastic base of an ideal character to assist in attaining the various objects of the invention as aforesaid, and also to facilitate the provision of 75 an ink pad proper at exceedingly low cost.

The sponge fibre employed with the moxa is desirably produced by combing the sponges used, as by any of the well known ginning or combing machines or devices, in such manner that small fibres are obtained. These fibres are preferably very small, even as compared in maximum dimension to the length of the familiar radially extended filamentous elements of the common swamp cat-tail,—which filamentous elements the moxa greatly resembles. True moxa, as is well known, is a soft, downy substance prepared in China and Japan from the young leaves of *Artemisia moxa*, and this is the moxa I 95 preferably employ, as the invention is at present understood.

In combination with the fibrous base, I employ a combination of liquids one at least of which is oleaginous in character, the latter 100

being preferably a drying vegetable oil; ideal results having been obtained so far with amoora oil.

In combination with the fibrous base and the oily binder just referred to, I further have found it desirable to employ, in addition to a dye, alcohol and glycerin.

The dye or dyes selected may be of any desired color or colors, chosen in accordance with a predetermination of the "working color" of the stamp pad proper, or equivalent. The dye or dyes employed, however, are preferably basic.

In the embodiment of the invention as at present preferred, the ingredients defined above are employed in the following proportions, approximately:

|              |          |
|--------------|----------|
| Sponge fibre | 100 lbs. |
| Alcohol      | 10 lbs.  |
| Glycerin     | 50 lbs.  |
| Oil          | 1 lb.    |
| Dye          | 1 lb.    |
| Moxa         | 10 lbs.  |

These ingredients, in the preferred embodiment of the invention, are handled as follows: The dye or dyes are dissolved in the glycerin and oil, the alcohol is thoroughly mixed in, and the resulting liquid is uniformly or substantially uniformly distributed over the surfaces and within the interstices and pores of the sponge fibre and moxa, in any suitable way, as by continued agitation of the fibres and liquid ingredients in a suitable vat or the like; the dissimilar fibres having previously been given a similar agitation, tossing or tumbling treatment to intimately commingle and substantially uniformly distribute the same. Where the fibres have been intermingled previously as last described, the vat agitation referred to may be reduced; and in some cases, where such preparatory fibre-intermingling is such as to result in an exceptionally uniform distribution of the dissimilar fibres, the previously mixed liquid ingredients may be chiefly or perhaps entirely added by way of a mere soaking operation.

The final result is a plastic mass or paste, ready to be spread within or upon a suitable support, as within a shallow tray, and there compressed. The degree of compression employed, applied in any suitable way, is such as to form a cake or layer of the desired thickness, and having about the same cushion characteristic as an ordinary cloth covered stamp pad proper, in fully "live", or new, condition. The degree of compression to be employed will quickly become ascertained in practice and be thereafter familiar in carrying out the manufacture of the new composition of matter; it being pointed out that the plastic mass is compressed to just short of the point where the liquid contents begin to exude noticeably.

In use, the new stamp pad proper, or equivalent, "gives" rather readily under the application of a type-carrying stamp or the like, the type or equivalents squeezing against the contacted and underlying fibres to receive the correct coating of dye or ink; and the inherent elasticity of the stamp pad proper, or equivalent, is such that the same restores itself to original form and surface height after each inking service.

The new composition of matter is inexpensive to manufacture; convenient to fabricate and shape or mount as above explained; and, as also already brought out, is adapted to attain all the objects and advantages of the invention hereinbefore recited, including also the avoidance of any chance of its having the useful life of a stamp pad proper or the like made therefrom impaired by wear and tear on a covering element of cloth, felt or the like, since there is no such covering element present.

What I claim as new, and desire to secure by Letters Patent, is:

A composition of matter forming an inking pad and resulting from mixing together the following: sponge fibre, one hundred pounds; moxa fibre, ten pounds; alcohol, ten pounds; glycerin, fifty pounds; oil, one pound; and dye, one pound.

In testimony whereof I hereby affix my signature.

TATSUO WAKABAYASHI.

90

95

100

105

110

115

120

125

130